



US011111456B2

(12) **United States Patent**  
Lee et al.

(10) **Patent No.:** US 11,111,456 B2  
(45) **Date of Patent:** Sep. 7, 2021

(54) **LUBRICANT COMPOSITION FOR HYDRAULIC OIL**

(71) Applicant: **DL Chemical CO., LTD.**, Seoul (KR)

(72) Inventors: **Hyeyung Jin Lee**, Daejeon (KR); **Jin Hun Ju**, Daejeon (KR)

(73) Assignee: **DL Chemical CO., LTD.**, Seoul (KR)

(\*) Notice: Subject to any disclaimer, the term of this patent is extended or adjusted under 35 U.S.C. 154(b) by 0 days.

(21) Appl. No.: **16/680,760**

(22) Filed: **Nov. 12, 2019**

(65) **Prior Publication Data**

US 2020/0277543 A1 Sep. 3, 2020

(30) **Foreign Application Priority Data**

Feb. 28, 2019 (KR) ..... 10-2019-0023681

(51) **Int. Cl.**

**C10M 169/04** (2006.01)  
**C10M 107/02** (2006.01)  
**C10M 137/10** (2006.01)  
**C10M 137/12** (2006.01)  
**C10M 143/02** (2006.01)  
**C10N 30/00** (2006.01)  
**C10N 30/06** (2006.01)  
**C10N 30/08** (2006.01)  
**C10N 30/10** (2006.01)  
**C10N 40/08** (2006.01)

(52) **U.S. Cl.**

CPC ..... **C10M 169/044** (2013.01); **C10M 107/02** (2013.01); **C10M 137/105** (2013.01); **C10M 137/12** (2013.01); **C10M 143/02** (2013.01); **C10M 2205/022** (2013.01); **C10M 2205/0206** (2013.01); **C10M 2223/047** (2013.01); **C10M 2223/06** (2013.01); **C10N 2030/06** (2013.01); **C10N 2030/08** (2013.01); **C10N 2030/10** (2013.01); **C10N 2030/40** (2020.05); **C10N 2040/08** (2013.01)

(58) **Field of Classification Search**

CPC ..... C10M 137/02; C10M 137/04; C10M 137/12; C10M 2223/02; C10M 2223/04; C10M 2223/06; C10M 169/044; C10M 107/02; C10M 137/105; C10M 143/02; C10M 2205/022; C10M 2223/047; C10M 2205/0206; C10N 2030/06; C10N 2040/08; C10N 2030/08; C10N 2030/10; C10N 2030/40

See application file for complete search history.

(56) **References Cited**

U.S. PATENT DOCUMENTS

|                  |         |                                 |
|------------------|---------|---------------------------------|
| 7,759,294 B2     | 7/2010  | Devlin et al.                   |
| 2014/0011720 A1  | 1/2014  | Antzutkin et al.                |
| 2014/0087986 A1* | 3/2014  | Patil ..... C10M 107/42 508/563 |
| 2015/0232777 A1  | 8/2015  | Qu et al.                       |
| 2016/0032214 A1  | 2/2016  | Shinoda et al.                  |
| 2016/0160148 A1  | 6/2016  | Rai                             |
| 2016/0304804 A1* | 10/2016 | Boesmann ..... C23F 11/167      |

FOREIGN PATENT DOCUMENTS

|    |                   |          |
|----|-------------------|----------|
| CN | 107148463 A       | 9/2017   |
| EP | 2 921 509 A1      | 9/2015   |
| JP | 2007-262300 A     | 10/2007  |
| JP | 2008-239687 A     | 10/2008  |
| JP | 2010-047735 A     | 3/2010   |
| JP | 2010-077390 A     | 4/2010   |
| JP | 2011-190377 A     | 9/2011   |
| JP | 2011190377 A      | * 9/2011 |
| JP | 2014-201737 A     | 10/2014  |
| KR | 10-0201759 B1     | 6/1999   |
| KR | 10-2008-0109015 A | 12/2008  |
| RU | 2500683 C2        | 12/2013  |

OTHER PUBLICATIONS

Search Report dated Mar. 18, 2020 from the Russian Federal Service for Intellectual Property in Application No. 2019136191/04. Decision on Grant of a Patent for Invention dated Jun. 18, 2020 from the Russian Federal Service for Intellectual Property in Application No. 2019136191/04.

Extended European Search Report dated Jun. 23, 2020 from the European Patent Office in Application No. 19207901.0.

Notice of Reasons for Refusal dated Dec. 8, 2020 from the Japanese Patent Office in Application No. 2019-204555.

\* cited by examiner

Primary Examiner — Taiwo Oladapo

(74) Attorney, Agent, or Firm — Sughrue Mion, PLLC

(57) **ABSTRACT**

The present invention relates to a lubricant composition, and more particularly to a lubricant composition, which has superior oxidation stability and friction characteristics even under harsh conditions of high temperature and high pressure and is thus suitable for use in hydraulic oil. The lubricant composition of the present invention includes a base oil, a liquid olefin copolymer, a phosphorothioate compound, and phosphonium phosphate.

11 Claims, No Drawings

**1**  
**LUBRICANT COMPOSITION FOR  
HYDRAULIC OIL**

CROSS-REFERENCE TO RELATED  
APPLICATIONS

This application is based on and claims priority from Korean Patent Application No. 10-2019-0023681, filed on Feb. 28, 2019 with the Korean Intellectual Property Office, the disclosure of which is incorporated herein in its entirety by reference.

BACKGROUND OF THE INVENTION

1. Technical Field

The present invention relates to a lubricant composition, and more particularly to a lubricant composition, which has superior oxidation stability and friction characteristics even under harsh conditions of high temperature and high pressure and is thus suitable for use in hydraulic oil.

2. Description of the Related Art

A lubricant is an oily material used to reduce the generation of frictional force on the friction surface of a machine or to dissipate frictional heat generated from the friction surface. Because of the wide variety of machinery that requires lubrication and the wide variety of conditions under which such machinery works, lubricants vary in type and quality. Depending on the application thereof, different types of base oil must be used. In particular, when a lubricant is used for an airplane or an advanced hydraulic system, hydraulic oil having a strong flame-retarding effect is required.

Any type of hydraulic oil used in industrial fields is a medium of power transmission and plays roles in lubrication, rust prevention, sealing and cooling of respective parts of hydraulic equipment. The hydraulic oil is manufactured by adding additives to base oil, and is largely classified into mineral hydraulic oil (petroleum-based hydraulic oil) and synthetic hydraulic oil depending on the type of base oil, synthetic hydraulic oil being classified into polyalphaolefin-based hydraulic oil and ester-based hydraulic oil.

Meanwhile, the operating temperature range of hydraulic oil varies, and especially in the summer, may be 75 to 850 or higher. At such temperatures, however, mineral hydraulic oil and polyalphaolefin-based hydraulic oil generate a lot of oil vapor. The occurrence of such oil vapor causes a problem of increasing the evaporation loss of hydraulic oil, and also promotes the oxidation of hydraulic oil. Hence, it is necessary to minimize the generation of oil vapor. In particular, mineral hydraulic oil, which accounts for most hydraulic oil, requires additional measures to improve oxidation stability due to the characteristics of the base feedstock oil. Moreover, since hydraulic systems are recently becoming more and more sophisticated, hydraulic oil is required to have superior friction characteristics.

Therefore, the present inventors have developed a lubricant composition for hydraulic oil, which has superior thermal and oxidation stability and is capable of reducing mechanical wear of hydraulic equipment.

CITATION LIST

Patent Literature

(Patent Document 0001) Korean Patent No. 10-0201759  
 (Patent Document 0002) Korean Patent Application Publication No. 10-2008-0109015

**2**  
**SUMMARY OF THE INVENTION**

Accordingly, the present invention has been made keeping in mind the problems encountered in the related art, and an objective of the present invention is to provide a lubricant composition, in which a functional additive for friction reduction and an ethylene-alphaolefin liquid random copolymer having a high viscosity index are mixed, thereby exhibiting superior friction characteristics, thermal stability and oxidation stability.

Another objective of the present invention is to provide a lubricant composition for hydraulic oil, which is capable of reducing the mechanical wear of hydraulic equipment and energy consumption when applied to hydraulic equipment and of decreasing evaporation loss due to low changes in the physical properties of hydraulic oil, and thus may be used for a long period of time.

In order to accomplish the above objectives, the present invention provides a lubricant composition, comprising a base oil, a liquid olefin copolymer, a phosphorothioate compound, and phosphonium phosphate.

The base oil may be at least one selected from the group consisting of mineral oil, polyalphaolefin (PAO) and ester.

The liquid olefin copolymer may be prepared by copolymerizing ethylene and alphaolefin in the presence of a single-site catalyst system, and the single-site catalyst system preferably includes a metallocene catalyst, an organometallic compound and an ionic compound.

The liquid olefin copolymer may have a coefficient of thermal expansion of 3.0 to 4.0.

The liquid olefin copolymer may be included in an amount of 0.5 to 30 wt %, and preferably 0.5 to 25 wt %, in the lubricant composition of the present invention.

The phosphorothioate compound may be included in an amount of 0.1 to 5.0 wt %, and preferably 0.1 to 3.0 wt %, in the lubricant composition.

The phosphonium phosphate may be included in an amount of 0.05 to 3.0 wt %, and preferably 0.1 to 1.5 wt %, in the lubricant composition.

The lubricant composition may have an SRV friction coefficient of 0.1 to 0.35 and a traction coefficient of 0.15 to 0.3.

According to the present invention, a lubricant composition includes phosphorothioate, phosphonium phosphate, and an ethylene-alphaolefin liquid random copolymer having a high viscosity index, which are mixed together, thereby improving friction characteristics and thermal and oxidation stability, and is capable of reducing the mechanical wear of hydraulic equipment and energy consumption when applied to hydraulic equipment, thereby maximizing energy-saving effects.

Also, according to the present invention, the lubricant composition has low changes in the physical properties of hydraulic oil, thus decreasing evaporation loss, and can endure 1000 min or more, and preferably 1200 min or more, in an RBOT oxidation stability test (ASTM D2271), thereby enabling the long-term use thereof as hydraulic oil.

DESCRIPTION OF SPECIFIC EMBODIMENTS

Hereinafter, a detailed description will be given of the present invention.

The present invention relates to a lubricant composition, which has superior oxidation stability and friction charac-

teristics and is thus suitable for use in hydraulic oil. Hence, the lubricant composition of the present invention includes a base oil, a liquid olefin copolymer, a phosphorothioate compound, and phosphonium phosphate.

Here, the base oil varies from the aspects of viscosity, heat resistance, oxidation stability and the like depending on the manufacturing method or refining method, but is generally classified into mineral oil and synthetic oil. The API (American Petroleum Institute) classifies base oil into five types, namely Group I, II, III, IV and V. These types, based on API ranges, are defined in API Publication 1509, 15<sup>th</sup> Edition, Appendix E, April 2002, and are shown in Table 1 below.

TABLE 1

|           | Saturated hydrocarbon (%) | Sulfur (%)              | Viscosity index |
|-----------|---------------------------|-------------------------|-----------------|
| Group I   | <90                       | >0.03                   | 80 ≤ VI < 120   |
| Group II  | ≥90                       | ≤0.03                   | 80 ≤ VI < 120   |
| Group III | ≥90                       | ≤0.03                   | VI ≥ 120        |
| Group IV  |                           | PAO (Poly Alpha Olefin) |                 |
| Group V   |                           | Ester & Others          |                 |

In the lubricant composition of the present invention, the base oil may be at least one selected from the group consisting of mineral oil, polyalphaolefin (PAO) and ester, and may be any type among Groups I to V based on the API ranges.

More specifically, mineral oil belongs to Groups I to III based on the API ranges, and mineral oil may include oil resulting from subjecting a lubricant distillate fraction, obtained through atmospheric distillation and/or vacuum distillation of crude oil, to at least one refining process of solvent deasphalting, solvent extraction, hydrogenolysis, solvent dewaxing, catalytic dewaxing, hydrorefining, sulfuric acid cleaning, and white clay treatment; wax isomerized mineral oil; or a gas-to-liquid (GLT) oil obtained via the Fischer-Tropsch process.

The synthetic oil belongs to Group IV or V based on the API ranges, and polyalphaolefin belonging to Group IV may be obtained through oligomerization of a higher alphaolefin using an acid catalyst, as disclosed in U.S. Pat. Nos. 3,780,128, 4,032,591, Japanese Patent Application Publication No. Hei. 1-163136, and the like, but the present invention is not limited thereto.

Examples of the synthetic oil belonging to Group V include alkyl benzenes, alkyl naphthalenes, isobutene oligomers or hydrides thereof, paraffins, polyoxy alkylene glycol, dialkyl diphenyl ether, polyphenyl ether, ester, and the like.

Here, the alkyl benzenes and alkyl naphthalenes are usually dialkylbenzene or dialkylnaphthalene having an alkyl chain length of 6 to 14 carbon atoms, and the alkyl benzenes or alkyl naphthalenes are prepared through Friedel-Crafts alkylation of benzene or naphthalene with olefin. The alkylated olefin used in the preparation of alkyl benzenes or alkyl naphthalenes may be linear or branched olefins or combinations thereof.

Also, examples of the ester include, but are not limited to, ditridecyl glutarate, di-2-ethylhexyl adipate, diisodecyl adipate, ditridecyl adipate, di-2-ethylhexyl sebacate, tridecyl pelargonate, di-2-ethylhexyl adipate, di-2-ethylhexyl azelate, trimethylolpropane caprylate, trimethylolpropane pelargonate, trimethylolpropane triheptanoate, pentaerythritol 2-ethylhexanoate, pentaerythritol pelargonate, pentaerythritol tetraheptanoate, and the like.

In the lubricant composition of the present invention, the liquid olefin copolymer is prepared by copolymerizing ethylene and alphaolefin monomers in the presence of a single-site catalyst system in order to uniformly distribute alphaolefin units in the copolymer chain. Preferably, the liquid olefin copolymer is prepared by reacting ethylene and alphaolefin monomers in the presence of a single-site catalyst system including a crosslinked metallocene compound, an organometallic compound, and an ionic compound for forming an ion pair through reaction with the crosslinked metallocene compound.

Here, the metallocene compound included in the single-site catalyst system may be at least one selected from the group consisting of Chemical Formulas 1 to 6 below.

[Chemical Formula 1]



[Chemical Formula 2]



[Chemical Formula 3]



**5**  
-continued

[Chemical Formula 4]



In Chemical Formulas 1 to 4,

M is a transition metal selected from the group consisting of titanium, zirconium, and hafnium,

B is absent or is a linking group including a C1-C20 alkylene group, a C6-C20 arylene group, C1-C20 dialkyl silicon, C1-C20 dialkyl germanium, a C1-C20 alkylphosphine group or a C1-C20 alkylamine group,

X<sub>1</sub> and X<sub>2</sub>, which are the same as or different from each other, are each independently a halogen atom, a C1-C20 alkyl group, a C2-C20 alkenyl group, a C2-C20 alkynyl group, a C6-C20 aryl group, a C7-C40 alkylaryl group, a C7-C40 arylalkyl group, a C1-C20 alkylamido group, a C6-C20 arylamido group, a C1-C20 alkylidene group or a C1-C20 alkoxy group, and

R<sub>1</sub> to R<sub>10</sub>, which are the same as or different from each other, are each independently hydrogen, a C1-C20 alkyl group, a C2-C20 alkenyl group, a C6-C20 aryl group, a C7-C20 alkylaryl group, a C7-C20 arylalkyl group, a C5-C60 cycloalkyl group, a C4-C20 heterocyclic group, a C1-C20 alkynyl group, a C6-C20-aryl-containing hetero group or a silyl group.

[Chemical Formula 5]



**6**  
-continued

[Chemical Formula 6]



In Chemical Formulas 5 and 6,

M is a transition metal selected from the group consisting of titanium, zirconium, and hafnium,

B is absent or is a linking group including a C1-C20 alkylene group, a C6-C20 arylene group, a C1-C20 dialkyl silicon, a C1-C20 dialkyl germanium, a C1-C20 alkylphosphine group or a C1-C20 alkylamine group,

X<sub>1</sub> and X<sub>2</sub>, which are the same as or different from each other, are each independently a halogen atom, a C1-C20 alkyl group, a C2-C20 alkenyl group, a C2-C20 alkynyl group, a C6-C20 aryl group, a C7-C40 alkylaryl group, a C7-C40 arylalkyl group, a C1-C20 alkylamido group, a C6-C20 arylamido group, a C1-C20 alkylidene group or a C1-C20 alkoxy group, and

R<sub>1</sub> to R<sub>10</sub>, which are the same as or different from each other, are each independently hydrogen, a C1-C20 alkyl group, a C2-C20 alkenyl group, a C6-C20 aryl group, a C7-C20 alkylaryl group, a C7-C20 arylalkyl group, a C5-C60 cycloalkyl group, a C4-C20 heterocyclic group, a C1-C20 alkynyl group, a C6-C20-aryl-containing hetero group or a silyl group.

Furthermore, all of R<sub>11</sub>, R<sub>13</sub> and R<sub>14</sub> are hydrogen, and each of R<sub>12</sub> radicals, which are the same as or different from each other, may independently be hydrogen, a C1-C20 alkyl group, a C2-C20 alkenyl group, a C6-C20 aryl group, a C7-C20 alkylaryl group, a C7-C20 arylalkyl group, a C5-C60 cycloalkyl group, a C4-C20 heterocyclic group, a C1-C20 alkynyl group, a C6-C20-aryl-containing hetero group or a silyl group.

Also, the metallocene compound of Chemical Formulas 2 to 6 may include a compound substituted through a hydroaddition reaction, and a preferred example thereof includes dimethylsilyl bis(tetrahydroindenyl) zirconium dichloride.

The organometallic compound included in the single-site catalyst system may be at least one selected from the group consisting of an organoaluminum compound, an organomagnesium compound, an organozinc compound and an organolithium compound, and is preferably an organoaluminum compound. The organoaluminum compound may be at least one selected from the group consisting of, for example, trimethylaluminum, triethylaluminum, triisobutylaluminum, tripropylaluminum, tributylaluminum, dimethylchloroaluminum, dimethylisobutylaluminum, dimethylethylaluminum, diethylchloroaluminum, triisopropylaluminum, triisobutylaluminum, tricyclopentylaluminum, tripentylaluminum, triisopentylaluminum, ethyl-

dimethylaluminum, methyldiethylaluminum, triphenylaluminum, methylaluminoxane, ethylaluminoxane, isobutylaluminoxane and butylaluminoxane, and is preferably triisobutylaluminum.

The ionic compound included in the single-site catalyst system may be at least one selected from the group consisting of organoboron compounds such as dimethylaluminum tetrakis(perfluorophenyl)borate, triphenylcarbenium tetrakis(perfluorophenyl)borate, and the like.

The component ratio of the single-site catalyst system may be determined in consideration of catalytic activity, and the molar ratio of metallocene catalyst:ionic compound: organometallic compound is preferably adjusted in the range of 1:1:5 to 1:10:1000 in order to ensure desired catalytic activity.

Furthermore, the components of the single-site catalyst system may be added at the same time or in any sequence to an appropriate solvent and may thus function as an active catalyst system. Here, the solvent may include, but is not limited to, a hydrocarbon solvent such as pentane, hexane, heptane, etc., or an aromatic solvent such as benzene, toluene, xylene, etc., and any solvent usable in the preparation may be used.

Also, the alphaolefin monomer used in the preparation of the liquid olefin copolymer includes a C2-C20 aliphatic olefin, and may specifically be at least one selected from the group consisting of ethylene, propylene, 1-butene, 1-pentene, 3-methyl-1-butene, 1-hexene, 4-methyl-1-pentene, 3-methyl-1-pentene, 1-heptene, 1-octene, 1-decene, 1-dodecene and 1-tetradecene, and may include isomeric forms, but the present invention is not limited thereto. In the copolymerization, the monomer content is 1 to 95 mol %, preferably 5 to 90 mol %.

The liquid olefin copolymer required in the present invention has a coefficient of thermal expansion of 3.0 to 4.0 and a bromine number of 0.1 or less.

The liquid olefin copolymer may be included in an amount of 0.5 to 30 wt %, and preferably 0.5 to 25 wt %, based on 100 wt % of the lubricant composition. If the amount of the liquid olefin copolymer is less than 0.5 wt % based on 100 wt % of the lubricant composition, stability may deteriorate. On the other hand, if the amount thereof exceeds 30 wt %, application of the resulting composition to hydraulic oil becomes difficult, which is undesirable.

The phosphorothioate compound, serving as a friction-reducing agent, may be at least one selected from the group consisting of monophosphorothioate, diphosphorothioate, triphosphorothioate, methylphosphorothioate, ethylphosphorothioate and sulfonylphosphorothioate. When the phosphorothioate compound is included in the lubricant composition, it may exhibit synergistic effects with an existing wear-resistant agent and friction reduction effects, and additionally, energy-saving effects may be achieved through friction reduction.

The phosphorothioate compound may be included in an amount of 0.1 to 5.0 wt %, and preferably 0.1 to 3.0 wt %, based on 100 wt % of the lubricant composition. If the amount of the phosphorothioate compound is less than 0.1 wt % based on 100 wt % of the lubricant composition, the friction reduction effect is insignificant. On the other hand, if the amount thereof exceeds 5.0 wt %, the additional reduction effect is insignificant despite the excessive addition thereof, which is undesirable.

The phosphonium phosphate is a material having the structure of Chemical Formula 7 below, and is used as a

friction/wear-reducing agent. In particular, when it is used together with the phosphorothioate compound, the effects thereof may be maximized.



The phosphonium phosphate exists in the form of an ionic liquid having both a phosphonium anion and a phosphate cation, and, among various phosphonium compounds, exhibits a characteristic friction/wear reduction effect.

Also, the phosphonium phosphate may be included in an amount of 0.05 to 3.0 wt %, and preferably 0.1 to 1.5 wt %, based on 100 wt % of the lubricant composition. If the amount of the phosphonium phosphate is less than 0.05 wt % based on 100 wt % of the lubricant composition, the friction/wear reduction effect may be insignificant. On the other hand, if the amount thereof exceeds 3.0 wt %, there is no synergistic effect thereof with the phosphorothioate compound, and wear may increase, which is undesirable.

The lubricant composition of the present invention may further include an additive selected from the group consisting of an antioxidant, a metal cleaner, an anticorrosive agent, a foam inhibitor, a pour-point depressant, a viscosity modifier, a wear-resistant agent and combinations thereof.

The antioxidant may be included in an amount of 0.01 to 5.0 wt % based on 100 wt % of the lubricant composition, and is preferably used in the form of a mixture of a phenolic antioxidant and an aminic antioxidant, more preferably a mixture of 0.01 to 3.0 wt % of the phenolic antioxidant and 0.01 to 3.0 wt % of the aminic antioxidant.

The phenolic antioxidant may be any one selected from the group consisting of 2,6-dibutylphenol, hindered bisphenol, high-molecular-weight hindered phenol, and hindered phenol with thioether.

The aminic antioxidant may be any one selected from the group consisting of diphenylamine, alkylated diphenylamine and naphthylamine, and preferably, the alkylated diphenylamine is dioctyldiphenylamine, octylated diphenylamine, or butylated diphenylamine.

The metal cleaner may be at least one selected from the group consisting of metallic phenate, metallic sulfonate, and metallic salicylate, and preferably, the metal cleaner is included in an amount of 0.1 to 10.0 wt % based on 100 wt % of the lubricant composition.

The anticorrosive agent may be a benzotriazole derivative, and is preferably any one selected from the group consisting of benzotriazole, 2-methylbenzotriazole, 2-phenylbenzotriazole, 2-ethylbenzotriazole and 2-propylbenzotriazole. The anticorrosive agent may be included in an amount of 0 to 4.0 wt % based on 100 wt % of the lubricant composition.

The foam inhibitor may be polyoxyalkylene polyol, and preferably, the foam inhibitor is included in an amount of 0 to 4.0 wt % based on 100 wt % of the lubricant composition.

The pour-point depressant may be poly(methacrylate), and preferably, the pour-point depressant is included in an amount of 0.01 to 5.0 wt % based on 100 wt % of the lubricant composition.

The viscosity modifier may be polyisobutylene or polymethacrylate, and preferably, the viscosity modifier is included in an amount of 0 to 15 wt % based on 100 wt % of the lubricant composition.

The wear-resistant agent may be at least one selected from the group consisting of organic borates, organic phosphites, organic sulfur-containing compounds, zinc dialkyl dithiophosphate, zinc diaryl dithiophosphate and phosphosulfurized hydrocarbon, and preferably, the wear-resistant agent is included in an amount of 0.01 to 3.0 wt %.

The lubricant composition of the present invention has an SRV friction coefficient of 0.1 to 0.35. Moreover, the lubricant composition has a traction coefficient of 0.15 to 0.3.

A better understanding of the present invention through the following examples. However, the present invention is not limited to these examples, but may be embodied in other forms. These examples are provided to thoroughly explain the invention and to sufficiently transfer the spirit of the present invention to those skilled in the art.

#### 1. Preparation of Additive Composition

An additive composition for use in the lubricant composition of the present invention was prepared as shown in Table 2 below.

TABLE 2

|                       | Additive composition         | Composition A | Composition B |
|-----------------------|------------------------------|---------------|---------------|
| Antioxidant           | 2,6-dibutylphenol            | 1             | 1.5           |
|                       | Diphenylamine                | 0.8           | 1             |
| Metal cleaner         | Metallic phenate             | 0.2           | 0.6           |
| Anticorrosive agent   | Benzotriazole                | 0.3           | 1.0           |
| Foam inhibitor        | Polyoxyalkylene polyol       | 0.01          | 0.02          |
| Pour-point depressant | Polymethacrylate             | 0.2           | 0.5           |
| Viscosity modifier    | Polyisobutylene              | —             | 1.0           |
| Wear-resistant agent  | Zinc dialkyl dithiophosphate | 0.2           | 1.1           |

#### 2. Preparation of Liquid Olefin Copolymer

A liquid olefin copolymer was prepared using an oligomerization method through a catalytic reaction process. Depending on the reaction time and conditions, which follow, liquid olefin copolymers having different molecular weights were prepared, and the properties thereof are shown in Table 3 below.

The reaction time and conditions were increased by 4 hr each from 20 hr. Here, the amounts of hydrogen and comonomer C3, which were added thereto, were increased by 10% each, and polymerization was performed under individual conditions, and the resulting polymers were classified depending on the molecular weight thereof.

TABLE 3

| 20            | Alphaolefin copolymer | Main properties      |                                    |                          |
|---------------|-----------------------|----------------------|------------------------------------|--------------------------|
|               |                       | Evaporation Loss (%) | Thickening Power (10 wt % in 150N) | CoE of Thermal Expansion |
| Copolymer I   | 1.28                  | 6                    | 3.00 to 3.20                       |                          |
| Copolymer II  | 0.54                  | 7                    | 3.20 to 3.40                       |                          |
| Copolymer III | 0.10                  | 8                    | 3.40 to 3.50                       |                          |
| Copolymer IV  | 0.001                 | 10                   | 3.50 to 3.60                       |                          |
| Copolymer V   | 0.0001                | 12                   | 3.60 to 3.70                       |                          |
| Copolymer VI  | 0.00001               | 14                   | 3.70 to 3.80                       |                          |

#### 30 3. Preparation of Lubricant Composition for Hydraulic Oil

A lubricant composition was prepared by mixing a base oil, the liquid olefin copolymer, a phosphorothioate compound, phosphonium phosphate and the additive prepared above, as shown in Tables 4 and 5 below. Here, the base oil was polyalphaolefin (PAO 4 cSt, available from Chevron Philips) having kinematic viscosity of 4 cSt at 1000, and the phosphorothioate compound was monophosphorothioate.

#### 35 Preparation Examples 1 to 67 and Comparative Examples 1 to 14. Lubricant Composition for Hydraulic Oil Including Additive A

TABLE 4

| Composition            | Base oil copolymer | Phosphorothioate Compound |                      | Phosphonium phosphate | Additive A |
|------------------------|--------------------|---------------------------|----------------------|-----------------------|------------|
|                        |                    | Alphaolefin               | Monophosphorothioate |                       |            |
| Preparation Example 1  | 97.135             | Copolymer I 0.05          | 0.1                  | 0.005                 | 2.71       |
| Preparation Example 2  | 96.735             | Copolymer I 0.05          | 0.5                  | 0.005                 | 2.71       |
| Preparation Example 3  | 95.74              | Copolymer I 0.05          | 1.0                  | 0.5                   | 2.71       |
| Preparation Example 4  | 93.74              | Copolymer I 0.05          | 3.0                  | 0.5                   | 2.71       |
| Preparation Example 5  | 88.74              | Copolymer I 0.05          | 5.0                  | 3.5                   | 2.71       |
| Preparation Example 6  | 96.64              | Copolymer I 0.5           | 0.1                  | 0.05                  | 2.71       |
| Preparation Example 7  | 95.74              | Copolymer I 0.5           | 1.0                  | 0.05                  | 2.71       |
| Preparation Example 8  | 93.69              | Copolymer I 0.5           | 3.0                  | 0.1                   | 2.71       |
| Preparation Example 9  | 92.09              | Copolymer I 5             | 0.1                  | 0.1                   | 2.71       |
| Preparation Example 10 | 91.69              | Copolymer I 5             | 0.5                  | 0.1                   | 2.71       |

TABLE 4-continued

| Composition            | Alphaolefin<br>Base oil copolymer | Phosphorothioate<br>Compound<br>Monophosphorothioate | Phosphonium<br>phosphate | Additive A |
|------------------------|-----------------------------------|------------------------------------------------------|--------------------------|------------|
| Preparation Example 11 | 89.19 Copolymer I 5               | 3.0                                                  | 0.1                      | 2.71       |
| Preparation Example 12 | 38.29 Copolymer I 5               | 5.0                                                  | 4.0                      | 2.71       |
| Preparation Example 13 | 86.89 Copolymer I 10              | 0.1                                                  | 0.3                      | 2.71       |
| Preparation Example 14 | 86.49 Copolymer I 10              | 0.5                                                  | 0.3                      | 2.71       |
| Preparation Example 15 | 85.99 Copolymer I 10              | 1.0                                                  | 0.3                      | 2.71       |
| Preparation Example 16 | 78.79 Copolymer I 10              | 5.0                                                  | 3.5                      | 2.71       |
| Preparation Example 17 | 76.69 Copolymer I 20              | 0.1                                                  | 0.5                      | 2.71       |
| Preparation Example 18 | 76.29 Copolymer I 20              | 0.5                                                  | 0.5                      | 2.71       |
| Preparation Example 19 | 70.29 Copolymer I 20              | 5.0                                                  | 2.0                      | 2.71       |
| Preparation Example 20 | 66.29 Copolymer I 30              | 0.5                                                  | 0.5                      | 2.71       |
| Preparation Example 21 | 60.79 Copolymer I 30              | 5.0                                                  | 1.5                      | 2.71       |
| Preparation Example 22 | 60.79 Copolymer I 35              | 0.5                                                  | 1.0                      | 2.71       |
| Preparation Example 23 | 61.19 Copolymer I 35              | 1.0                                                  | 0.1                      | 2.71       |
| Preparation Example 24 | 56.79 Copolymer I 35              | 3.0                                                  | 2.5                      | 2.71       |
| Preparation Example 25 | 53.79 Copolymer I 35              | 5.0                                                  | 3.5                      | 2.71       |
| Preparation Example 26 | 47.29 Copolymer I 35              | 10.0                                                 | 5.0                      | 2.71       |
| Preparation Example 27 | 47.235 Copolymer I 50             | 0.05                                                 | 0.005                    | 2.71       |
| Preparation Example 28 | 46.285 Copolymer I 50             | 1.0                                                  | 0.005                    | 2.71       |
| Preparation Example 29 | 38.79 Copolymer I 50              | 5.0                                                  | 3.5                      | 2.71       |
| Preparation Example 30 | 96.64 Copolymer II 0.05           | 0.1                                                  | 0.5                      | 2.71       |
| Preparation Example 31 | 95.24 Copolymer II 0.05           | 0.5                                                  | 1.5                      | 2.71       |
| Preparation Example 32 | 94.24 Copolymer II 0.05           | 1.0                                                  | 2.0                      | 2.71       |
| Preparation Example 33 | 92.24 Copolymer II 0.05           | 3.0                                                  | 2.0                      | 2.71       |
| Preparation Example 34 | 90.24 Copolymer II 0.05           | 5.0                                                  | 2.0                      | 2.71       |
| Preparation Example 35 | 96.19 Copolymer II 0.5            | 0.1                                                  | 0.5                      | 2.71       |
| Preparation Example 36 | 93.29 Copolymer II 0.5            | 3.0                                                  | 0.5                      | 2.71       |
| Preparation Example 37 | 83.79 Copolymer II 5              | 5.0                                                  | 3.5                      | 2.71       |
| Preparation Example 38 | 78.79 Copolymer II 10             | 5.0                                                  | 3.5                      | 2.71       |
| Preparation Example 39 | 72.285 Copolymer II 20            | 5.0                                                  | 0.005                    | 2.71       |
| Preparation Example 40 | 97.139 Copolymer III 0.05         | 0.1                                                  | 0.001                    | 2.71       |
| Preparation Example 41 | 95.24 Copolymer III 0.05          | 0.5                                                  | 1.5                      | 2.71       |
| Preparation Example 42 | 94.24 Copolymer III 0.05          | 1.0                                                  | 2.0                      | 2.71       |
| Preparation Example 43 | 92.24 Copolymer III 0.05          | 3.0                                                  | 2.0                      | 2.71       |
| Preparation Example 44 | 91.69 Copolymer III 5             | 0.1                                                  | 0.5                      | 2.71       |
| Preparation Example 45 | 91.29 Copolymer III 5             | 0.5                                                  | 0.5                      | 2.71       |
| Preparation Example 46 | 76.29 Copolymer III 20            | 0.5                                                  | 0.5                      | 2.71       |
| Preparation Example 47 | 75.29 Copolymer III 20            | 1.0                                                  | 1.0                      | 2.71       |
| Preparation Example 48 | 91.19 Copolymer IV 5              | 0.1                                                  | 1.0                      | 2.71       |

TABLE 4-continued

| Composition            | Base oil | Alphaolefins<br>copolymer | Phosphorothioate<br>Compound<br>Monophosphorothioate | Phosphonium<br>phosphate | Additive A |
|------------------------|----------|---------------------------|------------------------------------------------------|--------------------------|------------|
| Preparation Example 49 | 88.29    | Copolymer IV 5            | 3.0                                                  | 1.0                      | 2.71       |
| Preparation Example 50 | 76.69    | Copolymer IV 20           | 0.5                                                  | 0.1                      | 2.71       |
| Preparation Example 51 | 73.29    | Copolymer IV 20           | 3.0                                                  | 1.0                      | 2.71       |
| Preparation Example 52 | 92.09    | Copolymer V 5             | 0.1                                                  | 0.1                      | 2.71       |
| Preparation Example 53 | 91.69    | Copolymer V 5             | 0.5                                                  | 0.1                      | 2.71       |
| Preparation Example 54 | 78.79    | Copolymer V 10            | 5.0                                                  | 3.5                      | 2.71       |
| Preparation Example 55 | 77.14    | Copolymer V 20            | 0.1                                                  | 0.05                     | 2.71       |
| Preparation Example 56 | 76.69    | Copolymer V 20            | 0.5                                                  | 0.1                      | 2.71       |
| Preparation Example 57 | 68.79    | Copolymer V 20            | 5.0                                                  | 3.5                      | 2.71       |
| Preparation Example 58 | 45.79    | Copolymer V 50            | 1.0                                                  | 0.5                      | 2.71       |
| Preparation Example 59 | 43.79    | Copolymer V 50            | 3.0                                                  | 0.5                      | 2.71       |
| Preparation Example 60 | 42.289   | Copolymer V 50            | 5.0                                                  | 0.001                    | 2.71       |
| Preparation Example 61 | 93.64    | Copolymer VI 0.05         | 0.1                                                  | 3.5                      | 2.71       |
| Preparation Example 62 | 93.24    | Copolymer VI 0.05         | 0.5                                                  | 3.5                      | 2.71       |
| Preparation Example 63 | 92.74    | Copolymer VI 0.05         | 1.0                                                  | 3.5                      | 2.71       |
| Preparation Example 64 | 92.14    | Copolymer VI 5            | 0.1                                                  | 0.05                     | 2.71       |
| Preparation Example 65 | 91.69    | Copolymer VI 5            | 0.5                                                  | 0.1                      | 2.71       |
| Preparation Example 66 | 77.09    | Copolymer VI 20           | 0.1                                                  | 0.1                      | 2.71       |
| Preparation Example 67 | 76.29    | Copolymer VI 20           | 0.5                                                  | 0.5                      | 2.71       |
| Comparative Example 1  | 97.24    | Copolymer I 0.05          | —                                                    | —                        | 2.71       |
| Comparative Example 2  | 93.74    | Copolymer II 0.05         | —                                                    | 3.5                      | 2.71       |
| Comparative Example 3  | 87.29    | Copolymer II 10           | —                                                    | —                        | 2.71       |
| Comparative Example 4  | 73.29    | Copolymer II 20           | —                                                    | 4.0                      | 2.71       |
| Comparative Example 5  | 67.29    | Copolymer II 30           | —                                                    | —                        | 2.71       |
| Comparative Example 6  | 87.29    | Copolymer III 5           | 5.0                                                  | —                        | 2.71       |
| Comparative Example 7  | 82.29    | Copolymer III 10          | 5.0                                                  | —                        | 2.71       |
| Comparative Example 8  | 72.29    | Copolymer III 20          | 5.0                                                  | —                        | 2.71       |
| Comparative Example 9  | 88.79    | Copolymer IV 5            | —                                                    | 3.5                      | 2.71       |
| Comparative Example 10 | 87.29    | Copolymer IV 5            | 5.0                                                  | —                        | 2.71       |
| Comparative Example 11 | 82.29    | Copolymer IV 5            | 10.0                                                 | —                        | 2.71       |
| Comparative Example 12 | 63.79    | Copolymer V 30            | —                                                    | 3.5                      | 2.71       |
| Comparative Example 13 | 58.79    | Copolymer V 35            | —                                                    | 3.5                      | 2.71       |
| Comparative Example 14 | 93.74    | Copolymer VI 0.05         | —                                                    | 3.5                      | 2.71       |

Preparation Examples 68 to 116 and Comparative  
 Examples 15 to 53. Lubricant Composition for  
 Hydraulic Oil Including Additive B

TABLE 5

| Composition             | Alphaolefin<br>Base oil copolymer | Phosphorothioate<br>compound<br>Monophosphorothioate | Phosphonium<br>phosphate | Additive B |
|-------------------------|-----------------------------------|------------------------------------------------------|--------------------------|------------|
| Preparation Example 68  | 92.58 Copolymer I 0.5             | 0.1                                                  | 0.1                      | 6.72       |
| Preparation Example 69  | 92.18 Copolymer I 0.5             | 0.5                                                  | 0.1                      | 6.72       |
| Preparation Example 70  | 91.68 Copolymer I 0.5             | 1.0                                                  | 0.1                      | 6.72       |
| Preparation Example 71  | 88.08 Copolymer I 5               | 0.1                                                  | 0.1                      | 6.72       |
| Preparation Example 72  | 87.28 Copolymer I 5               | 0.5                                                  | 0.5                      | 6.72       |
| Preparation Example 73  | 86.78 Copolymer I 5               | 1.0                                                  | 0.5                      | 6.72       |
| Preparation Example 74  | 82.68 Copolymer I 10              | 0.1                                                  | 0.5                      | 6.72       |
| Preparation Example 75  | 81.78 Copolymer I 10              | 1.0                                                  | 0.5                      | 6.72       |
| Preparation Example 76  | 79.78 Copolymer I 10              | 3.0                                                  | 0.5                      | 6.72       |
| Preparation Example 77  | 73.08 Copolymer I 20              | 0.1                                                  | 0.1                      | 6.72       |
| Preparation Example 78  | 72.28 Copolymer I 20              | 0.5                                                  | 0.5                      | 6.72       |
| Preparation Example 79  | 71.78 Copolymer I 20              | 1.0                                                  | 0.5                      | 6.72       |
| Preparation Example 80  | 92.18 Copolymer II 0.5            | 0.1                                                  | 0.5                      | 6.72       |
| Preparation Example 81  | 88.78 Copolymer II 0.5            | 3.0                                                  | 1.0                      | 6.72       |
| Preparation Example 82  | 54.78 Copolymer II 30             | 5.0                                                  | 3.5                      | 6.72       |
| Preparation Example 83  | 93.08 Copolymer III 0.05          | 0.1                                                  | 0.05                     | 6.72       |
| Preparation Example 84  | 91.73 Copolymer III 0.05          | 0.5                                                  | 1.0                      | 6.72       |
| Preparation Example 85  | 91.23 Copolymer III 0.05          | 1.0                                                  | 1.0                      | 6.72       |
| Preparation Example 86  | 89.23 Copolymer III 0.05          | 3.0                                                  | 1.0                      | 6.72       |
| Preparation Example 87  | 86.68 Copolymer III 5             | 0.1                                                  | 1.5                      | 6.72       |
| Preparation Example 88  | 86.28 Copolymer III 5             | 0.5                                                  | 1.5                      | 6.72       |
| Preparation Example 89  | 79.78 Copolymer III 5             | 5.0                                                  | 3.5                      | 6.72       |
| Preparation Example 90  | 74.78 Copolymer III 10            | 5.0                                                  | 3.5                      | 6.72       |
| Preparation Example 91  | 71.28 Copolymer III 20            | 0.5                                                  | 1.5                      | 6.72       |
| Preparation Example 92  | 70.78 Copolymer III 20            | 1.0                                                  | 1.5                      | 6.72       |
| Preparation Example 93  | 34.78 Copolymer III 50            | 5.0                                                  | 3.5                      | 6.72       |
| Preparation Example 94  | 89.63 Copolymer IV 0.05           | 0.1                                                  | 3.5                      | 6.72       |
| Preparation Example 95  | 89.23 Copolymer IV 0.05           | 0.5                                                  | 3.5                      | 6.72       |
| Preparation Example 96  | 86.68 Copolymer IV 5              | 0.1                                                  | 1.5                      | 6.72       |
| Preparation Example 97  | 83.28 Copolymer IV 5              | 3.0                                                  | 2.0                      | 6.72       |
| Preparation Example 98  | 79.78 Copolymer IV 5              | 5.0                                                  | 3.5                      | 6.72       |
| Preparation Example 99  | 68.28 Copolymer IV 20             | 3.0                                                  | 2.0                      | 6.72       |
| Preparation Example 100 | 72.68 Copolymer IV 20             | 0.5                                                  | 0.1                      | 6.72       |
| Preparation Example 101 | 42.68 Copolymer IV 50             | 0.1                                                  | 0.5                      | 6.72       |
| Preparation Example 102 | 88.13 Copolymer V 5               | 0.1                                                  | 0.05                     | 6.72       |
| Preparation Example 103 | 87.73 Copolymer V 5               | 0.5                                                  | 0.05                     | 6.72       |

TABLE 5-continued

| Composition             | Alphaolefin<br>Base oil copolymer | Phosphorothioate<br>compound<br>Monophosphorothioate | Phosphonium<br>phosphate | Additive B |
|-------------------------|-----------------------------------|------------------------------------------------------|--------------------------|------------|
| Preparation Example 104 | 79.78 Copolymer V 5               | 5.0                                                  | 3.5                      | 6.72       |
| Preparation Example 105 | 74.78 Copolymer V 10              | 5.0                                                  | 3.5                      | 6.72       |
| Preparation Example 106 | 73.08 Copolymer V 20              | 0.1                                                  | 0.1                      | 6.72       |
| Preparation Example 107 | 71.78 Copolymer V 20              | 1.0                                                  | 0.5                      | 6.72       |
| Preparation Example 108 | 86.73 Copolymer VI 0.05           | 3.0                                                  | 3.5                      | 6.72       |
| Preparation Example 109 | 84.73 Copolymer VI 0.05           | 5.0                                                  | 3.5                      | 6.72       |
| Preparation Example 110 | 87.68 Copolymer VI 5              | 0.5                                                  | 0.1                      | 6.72       |
| Preparation Example 111 | 84.28 Copolymer VI 5              | 3.0                                                  | 1.0                      | 6.72       |
| Preparation Example 112 | 68.28 Copolymer VI 20             | 3.0                                                  | 2.0                      | 6.72       |
| Preparation Example 113 | 61.28 Copolymer VI 30             | 1.0                                                  | 1.0                      | 6.72       |
| Preparation Example 114 | 39.73 Copolymer VI 50             | 0.05                                                 | 3.5                      | 6.72       |
| Preparation Example 115 | 42.28 Copolymer VI 50             | 0.5                                                  | 0.5                      | 6.72       |
| Preparation Example 116 | 38.279 Copolymer VI 50            | 5.0                                                  | 0.001                    | 6.72       |
| Comparative Example 16  | 68.28 Copolymer III 20            | 5.0                                                  | —                        | 6.72       |
| Comparative Example 17  | 58.28 Copolymer III 30            | 5.0                                                  | —                        | 6.72       |
| Comparative Example 18  | 58.18 Copolymer III 35            | 0.1                                                  | —                        | 6.72       |
| Comparative Example 19  | 57.78 Copolymer III 35            | 0.5                                                  | —                        | 6.72       |
| Comparative Example 20  | 57.28 Copolymer III 35            | 1.0                                                  | —                        | 6.72       |
| Comparative Example 21  | 55.28 Copolymer III 35            | 3.0                                                  | —                        | 6.72       |
| Comparative Example 22  | 43.18 Copolymer III 50            | 0.1                                                  | —                        | 6.72       |
| Comparative Example 23  | 42.78 Copolymer III 50            | 0.5                                                  | —                        | 6.72       |
| Comparative Example 24  | 42.28 Copolymer III 50            | 1.0                                                  | —                        | 6.72       |
| Comparative Example 25  | 89.73 Copolymer IV 0.05           | —                                                    | 3.5                      | 6.72       |
| Comparative Example 26  | 92.23 Copolymer IV 0.05           | 1.0                                                  | —                        | 6.72       |
| Comparative Example 27  | 90.23 Copolymer IV 0.05           | 3.0                                                  | —                        | 6.72       |
| Comparative Example 28  | 88.23 Copolymer IV 0.05           | 5.0                                                  | —                        | 6.72       |
| Comparative Example 29  | 87.78 Copolymer IV 5              | —                                                    | 0.5                      | 6.72       |
| Comparative Example 30  | 78.28 Copolymer IV 5              | 10.0                                                 | —                        | 6.72       |
| Comparative Example 31  | 83.28 Copolymer IV 10             | —                                                    | —                        | 6.72       |
| Comparative Example 32  | 78.28 Copolymer IV 10             | 5.0                                                  | —                        | 6.72       |
| Comparative Example 33  | 39.78 Copolymer IV 50             | —                                                    | 3.5                      | 6.72       |
| Comparative Example 34  | 42.78 Copolymer IV 50             | 0.5                                                  | —                        | 6.72       |
| Comparative Example 35  | 42.28 Copolymer IV 50             | 1.0                                                  | —                        | 6.72       |
| Comparative Example 36  | 40.28 Copolymer IV 50             | 3.0                                                  | —                        | 6.72       |
| Comparative Example 37  | 38.28 Copolymer IV 50             | 5.0                                                  | —                        | 6.72       |
| Comparative Example 38  | 93.23 Copolymer V 0.05            | —                                                    | —                        | 6.72       |
| Comparative Example 39  | 93.13 Copolymer V 0.05            | 0.1                                                  | —                        | 6.72       |
| Comparative Example 40  | 92.73 Copolymer V 0.05            | 0.5                                                  | —                        | 6.72       |

TABLE 5-continued

| Composition            | Alphaolefin<br>Base oil copolymer | Phosphorothioate<br>compound<br>Monophosphorothioate | Phosphonium<br>phosphate | Additive B |
|------------------------|-----------------------------------|------------------------------------------------------|--------------------------|------------|
| Comparative Example 41 | 92.23 V 0.05                      | Copolymer                                            | 1.0                      | —          |
| Comparative Example 42 | 90.23 V 0.05                      | Copolymer                                            | 3.0                      | —          |
| Comparative Example 43 | 88.23 V 0.05                      | Copolymer                                            | 5.0                      | —          |
| Comparative Example 44 | 84.78 V 5                         | Copolymer                                            | —                        | 3.5        |
| Comparative Example 45 | 69.78 V 20                        | Copolymer                                            | —                        | 3.5        |
| Comparative Example 46 | 63.28 V 30                        | Copolymer                                            | —                        | —          |
| Comparative Example 47 | 88.28 VI 5                        | Copolymer                                            | —                        | —          |
| Comparative Example 48 | 78.28 VI 10                       | Copolymer                                            | 5.0                      | —          |
| Comparative Example 49 | 58.18 VI 35                       | Copolymer                                            | 0.1                      | —          |
| Comparative Example 50 | 57.78 VI 35                       | Copolymer                                            | 0.5                      | —          |
| Comparative Example 51 | 57.28 VI 35                       | Copolymer                                            | 1.0                      | —          |
| Comparative Example 52 | 55.28 VI 35                       | Copolymer                                            | 3.0                      | —          |
| Comparative Example 53 | 53.28 VI 35                       | Copolymer                                            | 5.0                      | —          |

## 4. Evaluation of Properties

The properties of the lubricant compositions prepared in Preparation Examples and Comparative Examples were measured as follows. The results are shown in Tables 6 and 7 below.

## Friction Coefficient

In the ball-on-disc mode, friction performance was evaluated by sequentially elevating the temperature in increments of 10°C from 40 to 120°C at 50 Hz and comparing the average friction coefficients at individual temperatures.

Here, the friction coefficient value decreases with an increase in effectiveness.

## Traction Coefficient

The traction coefficient was measured using an MTM instrument made by PCS Instruments. Here, the measurement conditions were fixed at 50N and SRR 50%, and friction and traction were observed depending on changes in temperature. The temperature was varied from 40 to 120°C, and the average values were compared.

## Wear Resistance

Four steel balls were subjected to friction with the lubricant composition for 60 min under conditions of 20 kg load, 1200 rpm, and 540, the sizes of wear scars were compared, and evaluation was carried out in accordance with ASTM D4172. Here, the wear scar (average wear scar diameter, µm) value decreases with an increase in effectiveness.

## Oxidation Stability

Oxidation stability was measured using an RBOT (Rotational Bomb Oxidation Test) meter in accordance with ASTM D2271.

TABLE 6

|                       | SRV Friction<br>Coefficient | MTM Traction<br>Coefficient | 4 Ball<br>Wear<br>(µm) | Oxidation<br>stability<br>(RBOT, min) |
|-----------------------|-----------------------------|-----------------------------|------------------------|---------------------------------------|
| Preparation Example 1 | 0.701                       | 0.598                       | 496                    | 610                                   |

TABLE 6-continued

|                        | SRV Friction<br>Coefficient | MTM Traction<br>Coefficient | 4 Ball<br>Wear<br>(µm) | Oxidation<br>stability<br>(RBOT, min) |
|------------------------|-----------------------------|-----------------------------|------------------------|---------------------------------------|
| Preparation Example 2  | 0.732                       | 0.569                       | 477                    | 654                                   |
| Preparation Example 3  | 0.734                       | 0.587                       | 432                    | 523                                   |
| Preparation Example 4  | 0.735                       | 0.544                       | 501                    | 320                                   |
| Preparation Example 5  | 0.712                       | 0.523                       | 665                    | 249                                   |
| Preparation Example 6  | 0.288                       | 0.221                       | 142                    | 1580                                  |
| Preparation Example 7  | 0.285                       | 0.200                       | 152                    | 1650                                  |
| Preparation Example 8  | 0.265                       | 0.236                       | 133                    | 1600                                  |
| Preparation Example 9  | 0.264                       | 0.219                       | 121                    | 1480                                  |
| Preparation Example 10 | 0.267                       | 0.211                       | 110                    | 2000                                  |
| Preparation Example 11 | 0.240                       | 0.236                       | 106                    | 2110                                  |
| Preparation Example 12 | 0.736                       | 0.569                       | 511                    | 333                                   |
| Preparation Example 13 | 0.246                       | 0.222                       | 116                    | 2420                                  |
| Preparation Example 14 | 0.239                       | 0.207                       | 123                    | 1840                                  |
| Preparation Example 15 | 0.257                       | 0.217                       | 140                    | 1680                                  |
| Preparation Example 16 | 0.745                       | 0.564                       | 522                    | 285                                   |
| Preparation Example 17 | 0.258                       | 0.213                       | 146                    | 1590                                  |
| Preparation Example 18 | 0.259                       | 0.243                       | 147                    | 1510                                  |
| Preparation Example 19 | 0.754                       | 0.555                       | 536                    | 278                                   |
| Preparation Example 20 | 0.264                       | 0.222                       | 149                    | 1540                                  |
| Preparation Example 21 | 0.768                       | 0.561                       | 555                    | 269                                   |

TABLE 6-continued

|                        | SRV Friction Coefficient | MTM Traction Coefficient | 4 Ball Wear (µm) | Oxidation stability (RBOT, min) |    |
|------------------------|--------------------------|--------------------------|------------------|---------------------------------|----|
| Preparation Example 22 | 0.769                    | 0.532                    | 622              | 298                             | 5  |
| Preparation Example 23 | 0.774                    | 0.512                    | 654              | 277                             |    |
| Preparation Example 24 | 0.744                    | 0.533                    | 635              | 279                             | 10 |
| Preparation Example 25 | 0.730                    | 0.612                    | 598              | 311                             |    |
| Preparation Example 26 | 0.741                    | 0.633                    | 590              | 312                             |    |
| Preparation Example 27 | 0.745                    | 0.654                    | 455              | 322                             | 15 |
| Preparation Example 28 | 0.756                    | 0.687                    | 478              | 388                             |    |
| Preparation Example 29 | 0.725                    | 0.698                    | 497              | 368                             |    |
| Preparation Example 30 | 0.76                     | 0.685                    | 518              | 384                             |    |
| Preparation Example 31 | 0.769                    | 0.696                    | 523              | 368                             | 20 |
| Preparation Example 32 | 0.778                    | 0.641                    | 537              | 321                             |    |
| Preparation Example 33 | 0.792                    | 0.621                    | 556              | 325                             |    |
| Preparation Example 34 | 0.791                    | 0.632                    | 631              | 387                             | 25 |
| Preparation Example 35 | 0.269                    | 0.219                    | 106              | 1650                            |    |
| Preparation Example 36 | 0.279                    | 0.245                    | 108              | 1440                            |    |
| Preparation Example 37 | 0.793                    | 0.612                    | 623              | 345                             | 30 |
| Preparation Example 38 | 0.797                    | 0.587                    | 647              | 388                             |    |
| Preparation Example 39 | 0.755                    | 0.555                    | 612              | 321                             |    |
| Preparation Example 40 | 0.702                    | 0.665                    | 678              | 654                             | 35 |
| Preparation Example 41 | 0.682                    | 0.610                    | 598              | 523                             |    |
| Preparation Example 42 | 0.713                    | 0.587                    | 599              | 320                             |    |
| Preparation Example 43 | 0.715                    | 0.588                    | 587              | 333                             | 40 |
| Preparation Example 44 | 0.257                    | 0.219                    | 185              | 1490                            |    |
| Preparation Example 45 | 0.259                    | 0.236                    | 168              | 2110                            |    |
| Preparation Example 46 | 0.278                    | 0.217                    | 135              | 1580                            | 45 |
| Preparation Example 47 | 0.279                    | 0.213                    | 108              | 1490                            |    |
| Preparation Example 48 | 0.284                    | 0.222                    | 154              | 1480                            |    |
| Preparation Example 49 | 0.231                    | 0.247                    | 163              | 2456                            | 50 |
| Preparation Example 50 | 0.247                    | 0.278                    | 169              | 2122                            |    |
| Preparation Example 51 | 0.264                    | 0.248                    | 185              | 2020                            |    |
| Preparation Example 52 | 0.255                    | 0.256                    | 154              | 1854                            | 55 |
| Preparation Example 53 | 0.254                    | 0.219                    | 165              | 1681                            |    |
| Preparation Example 54 | 0.678                    | 0.512                    | 655              | 279                             |    |
| Preparation Example 55 | 0.269                    | 0.213                    | 116              | 1610                            |    |
| Preparation Example 56 | 0.278                    | 0.243                    | 123              | 1440                            | 60 |
| Preparation Example 57 | 0.744                    | 0.587                    | 478              | 347                             |    |
| Preparation Example 58 | 0.623                    | 0.588                    | 676              | 348                             |    |
| Preparation Example 59 | 0.634                    | 0.521                    | 618              | 384                             | 65 |

TABLE 6-continued

|                        | SRV Friction Coefficient | MTM Traction Coefficient | 4 Ball Wear (µm) | Oxidation stability (RBOT, min) |
|------------------------|--------------------------|--------------------------|------------------|---------------------------------|
| Preparation Example 60 | 0.709                    | 0.569                    | 589              | 368                             |
| Preparation Example 61 | 0.745                    | 0.587                    | 599              | 348                             |
| Preparation Example 62 | 0.725                    | 0.555                    | 568              | 384                             |
| Preparation Example 63 | 0.756                    | 0.548                    | 534              | 368                             |
| Preparation Example 64 | 0.284                    | 0.236                    | 147              | 2410                            |
| Preparation Example 65 | 0.291                    | 0.245                    | 149              | 1810                            |
| Preparation Example 66 | 0.264                    | 0.247                    | 108              | 1560                            |
| Preparation Example 67 | 0.284                    | 0.256                    | 110              | 1540                            |
| Comparative Example 1  | 0.721                    | 0.589                    | 454              | 510                             |
| Comparative Example 2  | 0.759                    | 0.674                    | 505              | 348                             |
| Comparative Example 3  | 0.775                    | 0.555                    | 436              | 258                             |
| Comparative Example 4  | 0.811                    | 0.588                    | 698              | 412                             |
| Comparative Example 5  | 0.766                    | 0.672                    | 664              | 510                             |
| Comparative Example 6  | 0.716                    | 0.521                    | 499              | 285                             |
| Comparative Example 7  | 0.717                    | 0.569                    | 580              | 278                             |
| Comparative Example 8  | 0.726                    | 0.587                    | 590              | 269                             |
| Comparative Example 9  | 0.725                    | 0.611                    | 510              | 465                             |
| Comparative Example 10 | 0.691                    | 0.587                    | 651              | 419                             |
| Comparative Example 11 | 0.711                    | 0.547                    | 587              | 322                             |
| Comparative Example 12 | 0.68                     | 0.563                    | 636              | 249                             |
| Comparative Example 13 | 0.7                      | 0.587                    | 597              | 321                             |
| Comparative Example 14 | 0.716                    | 0.539                    | 498              | 396                             |
| TABLE 7                |                          |                          |                  |                                 |
|                        | SRV Friction Coefficient | MTM Traction Coefficient | 4 Ball Wear (µm) | Oxidation stability (RBOT, min) |
| Preparation Example 68 | 0.291                    | 0.219                    | 121              | 1660                            |
| Preparation Example 69 | 0.268                    | 0.209                    | 122              | 1640                            |
| Preparation Example 70 | 0.269                    | 0.236                    | 132              | 1490                            |
| Preparation Example 71 | 0.264                    | 0.221                    | 159              | 2020                            |
| Preparation Example 72 | 0.247                    | 0.200                    | 164              | 2110                            |
| Preparation Example 73 | 0.231                    | 0.236                    | 176              | 2030                            |
| Preparation Example 74 | 0.255                    | 0.219                    | 157              | 1650                            |
| Preparation Example 75 | 0.254                    | 0.211                    | 161              | 1580                            |
| Preparation Example 76 | 0.251                    | 0.236                    | 196              | 1490                            |
| Preparation Example 77 | 0.260                    | 0.222                    | 186              | 1910                            |
| Preparation Example 78 | 0.269                    | 0.207                    | 193              | 1480                            |

TABLE 7-continued

|                         | SRV Friction Coefficient | MTM Traction Coefficient | 4 Ball Wear (µm) | Oxidation stability (RBOT, min) |  |
|-------------------------|--------------------------|--------------------------|------------------|---------------------------------|--|
| Preparation Example 79  | 0.278                    | 0.222                    | 190              | 1650                            |  |
| Preparation Example 80  | 0.279                    | 0.219                    | 176              | 1680                            |  |
| Preparation Example 81  | 0.284                    | 0.245                    | 189              | 2020                            |  |
| Preparation Example 82  | 0.755                    | 0.587                    | 458              | 249                             |  |
| Preparation Example 83  | 0.798                    | 0.639                    | 655              | 346                             |  |
| Preparation Example 84  | 0.768                    | 0.589                    | 636              | 347                             |  |
| Preparation Example 85  | 0.736                    | 0.598                    | 664              | 258                             |  |
| Preparation Example 86  | 0.747                    | 0.569                    | 673              | 269                             |  |
| Preparation Example 87  | 0.231                    | 0.219                    | 152              | 1790                            |  |
| Preparation Example 88  | 0.255                    | 0.211                    | 169              | 1560                            |  |
| Preparation Example 89  | 0.822                    | 0.587                    | 676              | 287                             |  |
| Preparation Example 90  | 0.813                    | 0.544                    | 618              | 288                             |  |
| Preparation Example 91  | 0.279                    | 0.236                    | 147              | 2110                            |  |
| Preparation Example 92  | 0.278                    | 0.219                    | 146              | 2020                            |  |
| Preparation Example 93  | 0.713                    | 0.555                    | 591              | 412                             |  |
| Preparation Example 94  | 0.693                    | 0.548                    | 587              | 322                             |  |
| Preparation Example 95  | 0.704                    | 0.512                    | 541              | 368                             |  |
| Preparation Example 96  | 0.277                    | 0.245                    | 149              | 2030                            |  |
| Preparation Example 97  | 0.284                    | 0.209                    | 198              | 1650                            |  |
| Preparation Example 98  | 0.715                    | 0.555                    | 612              | 345                             |  |
| Preparation Example 99  | 0.269                    | 0.256                    | 110              | 1910                            |  |
| Preparation Example 100 | 0.264                    | 0.219                    | 121              | 1480                            |  |
| Preparation Example 101 | 0.722                    | 0.589                    | 676              | 610                             |  |
| Preparation Example 102 | 0.291                    | 0.236                    | 132              | 1680                            |  |
| Preparation Example 103 | 0.268                    | 0.221                    | 158              | 1480                            |  |
| Preparation Example 104 | 0.713                    | 0.532                    | 580              | 365                             |  |
| Preparation Example 105 | 0.645                    | 0.555                    | 589              | 285                             |  |
| Preparation Example 106 | 0.255                    | 0.236                    | 194              | 1610                            |  |
| Preparation Example 107 | 0.231                    | 0.211                    | 169              | 1854                            |  |
| Preparation Example 108 | 0.758                    | 0.512                    | 578              | 321                             |  |
| Preparation Example 109 | 0.759                    | 0.563                    | 579              | 325                             |  |
| Preparation Example 110 | 0.251                    | 0.207                    | 154              | 2080                            |  |
| Preparation Example 111 | 0.260                    | 0.234                    | 169              | 2130                            |  |
| Preparation Example 112 | 0.261                    | 0.226                    | 226              | 1780                            |  |
| Preparation Example 113 | 0.275                    | 0.217                    | 169              | 1790                            |  |
| Preparation Example 114 | 0.813                    | 0.613                    | 501              | 415                             |  |
| Preparation Example 115 | 0.734                    | 0.580                    | 512              | 369                             |  |
| Preparation Example 116 | 0.784                    | 0.571                    | 523              | 358                             |  |

TABLE 7-continued

|                          | SRV Friction Coefficient | MTM Traction Coefficient | 4 Ball Wear (µm) | Oxidation stability (RBOT, min) |
|--------------------------|--------------------------|--------------------------|------------------|---------------------------------|
| 5 Comparative Example 16 | 0.702                    | 0.569                    | 589              | 299                             |
| Comparative Example 17   | 0.682                    | 0.564                    | 597              | 388                             |
| Comparative Example 18   | 0.726                    | 0.512                    | 478              | 347                             |
| Comparative Example 19   | 0.735                    | 0.533                    | 436              | 321                             |
| Comparative Example 20   | 0.749                    | 0.523                    | 505              | 247                             |
| Comparative Example 21   | 0.748                    | 0.532                    | 518              | 258                             |
| Comparative Example 22   | 0.725                    | 0.621                    | 556              | 401                             |
| Comparative Example 23   | 0.704                    | 0.633                    | 623              | 369                             |
| Comparative Example 24   | 0.779                    | 0.666                    | 655              | 358                             |
| Comparative Example 25   | 0.725                    | 0.555                    | 651              | 269                             |
| Comparative Example 26   | 0.779                    | 0.563                    | 523              | 388                             |
| Comparative Example 27   | 0.77                     | 0.611                    | 498              | 396                             |
| Comparative Example 28   | 0.691                    | 0.587                    | 599              | 348                             |
| Comparative Example 29   | 0.711                    | 0.588                    | 568              | 384                             |
| Comparative Example 30   | 0.716                    | 0.672                    | 647              | 346                             |
| Comparative Example 31   | 0.717                    | 0.499                    | 698              | 347                             |
| Comparative Example 32   | 0.745                    | 0.623                    | 612              | 299                             |
| Comparative Example 33   | 0.711                    | 0.639                    | 673              | 519                             |
| Comparative Example 34   | 0.702                    | 0.598                    | 618              | 654                             |
| Comparative Example 35   | 0.632                    | 0.569                    | 589              | 523                             |
| Comparative Example 36   | 0.612                    | 0.587                    | 597              | 320                             |
| Comparative Example 37   | 0.643                    | 0.547                    | 591              | 333                             |
| Comparative Example 38   | 0.756                    | 0.610                    | 698              | 412                             |
| Comparative Example 39   | 0.758                    | 0.600                    | 678              | 415                             |
| Comparative Example 40   | 0.759                    | 0.588                    | 598              | 369                             |
| Comparative Example 41   | 0.76                     | 0.541                    | 599              | 358                             |
| Comparative Example 42   | 0.769                    | 0.563                    | 587              | 347                             |
| Comparative Example 43   | 0.778                    | 0.522                    | 499              | 321                             |
| Comparative Example 44   | 0.715                    | 0.543                    | 590              | 399                             |
| Comparative Example 45   | 0.749                    | 0.555                    | 587              | 321                             |
| Comparative Example 46   | 0.646                    | 0.569                    | 523              | 278                             |
| Comparative Example 47   | 0.76                     | 0.611                    | 624              | 387                             |
| Comparative Example 48   | 0.822                    | 0.601                    | 444              | 412                             |
| Comparative Example 49   | 0.769                    | 0.587                    | 584              | 345                             |
| Comparative Example 50   | 0.778                    | 0.588                    | 562              | 346                             |
| Comparative Example 51   | 0.792                    | 0.541                    | 532              | 347                             |
| Comparative Example 52   | 0.791                    | 0.513                    | 521              | 258                             |

25

TABLE 7-continued

|                        | SRV Friction Coefficient | MTM Traction Coefficient | 4 Ball Wear ( $\mu\text{m}$ ) | Oxidation stability (RBOT, min) |
|------------------------|--------------------------|--------------------------|-------------------------------|---------------------------------|
| Comparative Example 53 | 0.793                    | 0.555                    | 511                           | 269                             |

As is apparent from Tables 6 and 7, the lubricant compositions including the liquid ethylene alphaolefin copolymer, the phosphorothioate compound and the phosphonium phosphate within the amount ranges of the present invention were significantly reduced in wear scar and friction coefficient compared to the lubricant compositions of Comparative Examples, and also exhibited superior oxidation stability. Therefore, it is concluded that the lubricant composition of the present invention is improved from the aspects of friction characteristics and stability and thus is suitable for use in hydraulic oil.

Although the embodiments of the present invention have been disclosed for illustrative purposes, those skilled in the art will appreciate that various modifications, additions and substitutions are possible, without departing from the scope and spirit of the invention as disclosed in the accompanying claims.

What is claimed is:

1. A lubricant composition, comprising:  
61.28 to 96.64% by weight of a base oil, 0.5 to 30% by weight of a liquid olefin copolymer, 0.1 to 3% by weight of a phosphorothioate compound, and 0.05 to 2% by weight of phosphonium phosphate,  
wherein the phosphorothioate compound is at least one selected from the group consisting of monophosphorothioate, diphenylphosphorothioate, triphenylphosphorothioate, methylphenylphosphorothioate, ethylphenylphosphorothioate, and sulfonylphenylphosphorothioate, and  
wherein the phosphonium phosphate has a structure of  
Chemical Formula 7 below

26

### [Chemical Formula 7]



2. The lubricant composition of claim 1, wherein the liquid olefin copolymer is prepared by copolymerizing ethylene and alphaolefin using a single-site catalyst system.

3. The lubricant composition of claim 2, wherein the single-site catalyst system includes a metallocene catalyst, an organometallic compound and an ionic compound.

4. The lubricant composition of claim 1, wherein the liquid olefin copolymer has a coefficient of thermal expansion of 3.0 to 4.0.

5. The lubricant composition of claim 1, wherein the liquid olefin copolymer has a bromine number of 0.1 or less.

6. The lubricant composition of claim 1, wherein the base oil is at least one selected from the group consisting of mineral oil, polyalphaolefin (PAO), and ester.

7. The lubricant composition of claim 1, further comprising an additive selected from the group consisting of an antioxidant, a metal cleaner, an anticorrosive agent, a foam inhibitor, a pour-point depressant, a viscosity modifier, a wear-resistant agent, and combinations thereof.

8. The lubricant composition of claim 1, wherein the lubricant composition has an SRV friction coefficient of 0.1 to 0.35.

9. The lubricant composition of claim 1, wherein the lubricant composition has a traction coefficient of 0.15 to 0.3.

10. The lubricant composition of claim 1, wherein the lubricant composition endures 1000 min or more in an oxidation stability evaluation (RBOT, ASTM D2271).

11. The lubricant composition of claim 1, wherein the lubricant composition is used as hydraulic oil.

\* \* \* \*